

Oct. 12, 1943.

G. F. NADEAU ET AL

2,331,717

PHOTOGRAPHIC FILM

Filed Nov. 26, 1940

FIG. 1



FIG. 2



FIG. 3



FIG. 4



GALE F. NADEAU  
CLEMENS B. STARCK  
INVENTORS

BY *Newton M. Perrine*  
*R. Frank Smith*  
ATTORNEYS

## UNITED STATES PATENT OFFICE

2,331,717

## PHOTOGRAPHIC FILM

Gale F. Nadeau and Clemens B. Starck, Rochester, N. Y., assignors to Eastman Kodak Company, Rochester, N. Y., a corporation of New Jersey

Application November 26, 1940, Serial No. 367,178

14 Claims. (Cl. 95—9)

This invention relates to a method for subbing photographic film and particularly to a sub for film designed to receive a colored photographic image.

The problem of producing a satisfactory safety film base possessing satisfactory stripping and brittleness qualities has been extremely difficult to solve. In order to cause photographic emulsion layers to adhere to cellulose organic acid ester supports, it is necessary to use intervening layers of such a character that the several layers do not strip from the support when the film is used or when the film is passed through processing baths, and also of such character that the layers do not adhere with such firmness that the film becomes brittle. One successful way of making a photographic film having satisfactory stripping and brittleness is to use a synthetic resinous material as a sub or undercoat as described in Nadeau U. S. Patent 2,133,110 granted October 11, 1938. The problem of causing a photographic emulsion to adhere to cellulose inorganic acid ester supports such as cellulose nitrate is not difficult, since it is necessary only to employ a simple gelatin sub on the cellulose nitrate support and overcoat with the usual gelatino-silver halide emulsion.

In the case of photographic film having an emulsion layer or several emulsion layers sensitized to record different regions of the spectrum and designed to receive colored images the subbing or undercoat layers must possess additional qualities. The dye or other coloring material used in the emulsion layers is likely to stain the sub coat if it is not properly constructed and the sub coat may cause a fading of the dye in the emulsion layer of the film next to the sub, when the film is incubated or stored. One method of preventing the retention of dye in a sub coat consists of using for this coating a mixture of a cellulose ester and a resin as described in a prior patent, Nadeau U. S. 2,169,004, granted August 8, 1939. Other methods which might appear to alleviate the condition of dye retention in subbing layers involve the use of mixed gelatin and synthetic resin subbing layers, as described in the prior U. S. patents, Babcock 2,096,675, Nadeau 2,096,616 and 2,096,617, all granted October 19, 1937. These methods, while representing an approach in the right direction do not entirely solve the problem inasmuch as some dyes tend to be retained in subbing layers, constructed according to the prior art, after processing a color film by well known methods. In addition it has been determined that films subbed with layers of material either containing an aldehyde or a material capable of decomposition into an aldehyde will show significantly high fog upon development.

The object of the present invention is to provide a subbing layer for a photographic film hav-

ing an emulsion layer or layers designed to receive colored images, which does not retain a dye stain caused by the colored image or dyes present in the film or formed during color processing operations. A further object is to provide a subbing layer which imparts satisfactory physical properties to a film. A still further object is to provide a photographic film with a subbing layer which is free of fog-producing substances.

These objects are accomplished in the present invention by providing a subbing layer consisting of a mixture of gelatin and a polymeric material, such as a polyvinyl ester, free from aldehyde or aldehyde-forming substances.

In the accompanying drawing Figs. 1, 2, 3 and 4 are enlarged sectional views of a photographic film having subbing layers thereon according to our invention.

In subbing film according to our invention a cellulose derivative support is coated with a subbing layer of gelatin and a polyvinyl ester. The support may consist of cellulose organic acid esters and mixed esters such as cellulose acetate or acetate propionate and cellulose inorganic acid esters such as cellulose nitrate. The polyvinyl ester of the subbing layer may be a fully esterified ester such as polyvinyl acetate, polyvinyl propionate, polyvinyl butyrate or a partially hydrolyzed polyvinyl ester. These polyvinyl esters are prepared by the esterification of polyvinyl alcohol, although it is questionable whether completely esterified polyvinyl esters are produced by this method. Otherwise a monomeric vinyl ester is polymerized to the polyvinyl ester and from this by hydrolysis may be prepared a partially hydrolyzed polyvinyl ester. The polyvinyl acetate we generally use is known under the trade name "Gelva," the preparation of which is described in U. S. patents, Klatte and Rollett 1,241,738, granted October 2, 1917; Herrmann et al. 1,586,803, granted June 1, 1926, and 1,710,825, granted April 30, 1929. We prefer to use the lower viscosity polymers prepared by these methods known as Gelva V-15, V-25 or V-30. Other resins which are suitable for use in the subbing layers of our invention in conjunction with gelatin but which are not generally as effective in the reduction of dye stain, are polyvinyl formaldehyde and acetaldehyde acetals and the esters of polyacrylic acid. After the application of the subbing layer of our invention to a support the sensitive emulsion layer or layers are coated thereupon usually without the interposition of any intervening adhesive layers. We prefer, however, in the case of mixed cellulose organic acid ester supports, first to sub the support with a hydrolyzed cellulose ester layer or, by a cellulose nitrate or mixed cellulose nitrate and polyvinyl ester layer, then the gelatin and polyvinyl ester layer, and finally the emulsion.

Cellulose nitrate and cellulose acetate supports may be subbed by an alternative method. We first coat the support with a cellulose nitrate or mixed cellulose nitrate and polyvinyl acetate layer followed by the mixed gelatin and polyvinyl ester subbing layer of our invention and one or more emulsion layers.

Our invention will now be described by particular reference to the accompanying drawing.

As shown in Fig. 1 a cellulose ester support 10 is subbed with a mixture of gelatin and a polymeric material free from aldehyde, e. g., gelatin and polyvinyl ester layer 11. The emulsion layer 12 is coated over the subbing layer 11.

As shown in Fig. 2 a cellulose nitrate support 10 is subbed with a mixed gelatin and polyvinyl acetate layer 11 and over this layer is coated the emulsion layer 12.

As shown in Fig. 3 a cellulose acetate support 10 is subbed with cellulose nitrate or mixed cellulose nitrate and polyvinyl acetate layer 13 followed by the mixed gelatin and polyvinyl acetate subbing layer 14 and the emulsion layer 12.

As shown in Fig. 4 a color film sensitized to record different regions of the spectrum consists of a cellulose acetate propionate support 10 and in order thereupon a cellulose nitrate or mixed cellulose nitrate and polyvinyl acetate layer 13, the mixed gelatin and polyvinyl acetate layer 11, and the red, green, and blue light sensitive emulsion layers 15, 16 and 17.

The method of subbing film according to our invention will now be illustrated by examples, it being understood that these are illustrative only.

#### Example 1

A cellulose nitrate film support was coated with the following subbing solution to which had been added 10-30% of the weight of the gelatin of polyvinyl acetate of low viscosity.

|             | Per cent |
|-------------|----------|
| Gelatin     | 0.6      |
| Acetone     | 39.0     |
| Water       | 6.0      |
| Methanol    | 53.4     |
| Acetic acid | 1.0      |

Over this layer was coated an ordinary emulsion layer. This film had satisfactory physical characteristics such as flexibility without brittleness and when a colored image was formed in the emulsion layer the subbing layer did not retain any dye.

#### Example 2

A cellulose nitrate film support was coated with the following subbing solution.

|                                                                     | Per cent |
|---------------------------------------------------------------------|----------|
| Cellulose nitrate (80-90% soluble in alcohol, low viscosity, 11% N) | 2.5      |
| Polyvinyl acetate                                                   | 0.6      |
| Acetone                                                             | 35.0     |
| Methanol                                                            | 56.9     |
| Butyl alcohol                                                       | 5.0      |

This solution was coated at a linear speed of 6 feet per minute and was dried after coating. A mixed gelatin and polyvinyl acetate subbing layer was then applied from a solution of the following composition:

|          | Per cent |
|----------|----------|
| Gelatin  | 1.2      |
| Water    | 10.0     |
| Acetone  | 35.0     |
| Methanol | 53.8     |

to which had been added 10-30% of the weight of gelatin of polyvinyl acetate. The water content of this formula may be varied from 5-20% and the acetone content from 0-70% in which cases the balance of the solvent is methanol. Over the gelatin and polyvinyl acetate layer was then coated a silver halide emulsion layer.

#### Example 3

10 A film support of cellulose acetate, 38-42% acetyl, was coated with a subbing solution of the following composition:

|                   | Per cent |
|-------------------|----------|
| Gelatin           | 1.2      |
| Acetone           | 69.0     |
| Water             | 8.0      |
| Methyl cellosolve | 5.0      |
| Methanol          | 15.8     |
| Acetic acid       | 1.0      |

20 to which 2% of the weight of gelatin of chromium chloride and 10-30% of the weight of the gelatin of polyvinyl acetate had been added. The use of chromium chloride in gelatin subbing layers has been described in our prior

25 application Serial No. 295,268. Over the mixed gelatin and polyvinyl acetate layer was then coated a silver halide emulsion.

By an alternative method we have first subbed a cellulose acetate base, 38-42% acetyl, with a mixed cellulose nitrate and polyvinyl acetate subbing layer from a solution such as described in Example 2 after which was applied a mixed gelatin and polyvinyl acetate subbing solution of the following composition

|             | Per cent |
|-------------|----------|
| Gelatin     | 1.2      |
| Water       | 10.0     |
| Methanol    | 87.8     |
| Acetic acid | 1.0      |

40 to which 10-30% of the weight of the gelatin of polyvinyl acetate was added. The water content of this formula may vary from 5-20% in which case the methanol content is varied accordingly. Over the gelatin and polyvinyl acetate layer was coated a sensitive emulsion layer.

#### Example 4

50 A film support of cellulose acetate propionate 16% propionyl and 30% acetyl was coated with a cellulose acetate propionate solution consisting of a mixture of 60% hydrolyzed cellulose acetate propionate, 10% propionyl and 23% acetyl, and 40% of hydrolyzed cellulose acetate propionate, 10% propionyl and 29% acetyl in a manner similar to that described in our prior application Serial No. 295,268 from a solution of the following composition

|                   | Per cent |
|-------------------|----------|
| Cellulose ester   | 2        |
| Methyl cellosolve | 25       |
| Acetone           | 35       |
| Methanol          | 33       |
| Ethylene chloride | 5        |

65 Over this sub layer was coated a layer of mixed gelatin and polyvinyl acetate from a solution of the composition which follows:

|                   | Per cent |
|-------------------|----------|
| Gelatin           | 1.2      |
| Acetone           | 59.0     |
| Water             | 8.0      |
| Methyl cellosolve | 10.0     |
| Methanol          | 20.8     |
| Acetic acid       | 1.0      |

75 to which was added 2% of the weight of the gela-

tin of chromium chloride and 10-30% of the weight of the gelatin of polyvinyl acetate. Over this subbing layer was then coated an emulsion layer.

*Example 5*

A film support of cellulose acetate propionate 16%, propionyl and 30% acetyl, was coated with a layer consisting of mixed cellulose nitrate and polyvinyl acetate from a subbing solution of the composition shown in Example 2, followed by the mixed gelatin and polyvinyl acetate subbing layer of the invention coated from a solution of the following composition:

|             | Per cent |
|-------------|----------|
| Gelatin     | 1.2      |
| Water       | 10.0     |
| Methanol    | 87.8     |
| Acetic acid | 1.0      |

to which was added 10-30% of the weight of the gelatin of polyvinyl acetate. The water content of this formula may vary from 5-20% in which case the amount of methanol is decreased. Over this subbing layer were coated several emulsion layers sensitized to record different regions of the spectrum. When this film was color processed it was found that no dye had been retained in the subbing layers or the support.

We have referred to the use of our subbing method in film designed to receive color images. Film support may also be subbed according to our invention where the film is designed to record black-and-white silver images. The color films we describe may be designed to record sound as well as picture images and suitable light filtering layers may be positioned throughout the film as is required.

It is to be understood that the above examples, ranges and methods of procedure are illustrative only and that our invention is to be taken as limited only by the scope of the appended claims.

Having thus described our invention what we claim as new and wish to secure by Letters Patent of the United States is:

1. A photographic film having low dye retention subbing layers, comprising a cellulose ester support, an emulsion layer adapted to receive a colored image, and between the emulsion and the support a subbing layer composed of a mixture of gelatin and a polymeric material selected from the group consisting of polyvinyl organic acid esters, hydrolyzed polyvinyl organic acid esters, polyacrylic esters and polyvinyl acetals.

2. A photographic film having low dye retention subbing layers, comprising a cellulose ester support, an emulsion layer adapted to receive a colored image and between the emulsion and the support, a subbing layer composed of a mixture of gelatin and a polyvinyl organic acid ester.

3. A photographic film for use in color photography having low dye retention subbing layers, comprising a cellulose organic acid ester support, an emulsion layer adapted to receive a colored image, and between the emulsion and the support, a subbing layer composed of a mixture of gelatin and a polyvinyl organic acid ester.

4. A photographic film for use in color photography having low dye retention subbing layers, comprising a cellulose acetate support, an emulsion layer adapted to receive a colored image, and between the emulsion and the support, a subbing layer composed of a mixture of the gelatin and a polyvinyl organic acid ester.

5. A photographic film for use in color photo-

tography having low dye retention subbing layers, comprising a cellulose acetate support, an emulsion layer adapted to receive a colored image, and between the emulsion and the support, a subbing layer composed of a mixture of gelatin and polyvinyl acetate.

6. A photographic film for use in color photography having low dye retention subbing layers, comprising a cellulose mixed ester support, an emulsion layer adapted to receive a colored image, and between the emulsion and the support, a subbing layer composed of a mixture of gelatin and a polyvinyl organic acid ester.

7. A photographic film for use in color photography having low dye retention subbing layers, comprising a cellulose acetate propionate support, an emulsion layer adapted to receive a colored image, and between the emulsion and the support, a subbing layer composed of a mixture of gelatin and a polyvinyl organic acid ester.

8. A photographic film for use in color photography having low dye retention subbing layers, comprising a cellulose acetate propionate support, an emulsion layer adapted to receive a colored image, and between the emulsion and the support, a subbing layer composed of a mixture of gelatin and polyvinyl acetate.

9. A photographic film for use in color photography having low dye retention subbing layers, comprising a cellulose inorganic acid ester support, an emulsion layer adapted to receive a colored image, and between the emulsion and the support, a subbing layer composed of a mixture of gelatin and a polyvinyl organic acid ester.

10. A photographic film for use in color photography having low dye retention subbing layers, comprising a cellulose nitrate support, an emulsion layer adapted to receive a colored image, and between the emulsion and the support, a subbing layer composed of a mixture of gelatin and a polyvinyl organic acid ester.

11. A photographic film for use in color photography having low dye retention subbing layers, comprising a cellulose nitrate support, an emulsion layer adapted to receive a colored image, and between the emulsion and the support, a subbing layer composed of a mixture of gelatin and polyvinyl acetate.

12. A photographic film for use in color photography having low dye retention subbing layers, comprising a cellulose nitrate support, an emulsion layer adapted to receive a colored image, and between the emulsion and the support, a subbing layer composed of a mixture of gelatin and partially hydrolyzed polyvinyl acetate.

13. A photographic film for use in color photography having low dye retention subbing layers comprising a cellulose acetate support, a plurality of emulsion layers sensitized to record different regions of the spectrum, and between the emulsions and the support, a subbing layer composed of a mixture of gelatin and polyvinyl acetate.

14. A photographic film for use in color photography having low dye retention subbing layers, comprising a cellulose acetate propionate support, a plurality of emulsion layers sensitized to record different regions of the spectrum, and between the emulsions and the support, a subbing layer composed of a mixture of gelatin and polyvinyl acetate.

GALE F. NADEAU.  
CLEMENS B. STARCK.